



US009181140B1

(12) **United States Patent**  
**Hamilton et al.**

(10) **Patent No.:** **US 9,181,140 B1**  
(45) **Date of Patent:** **Nov. 10, 2015**

(54) **SOLID PROPELLANT BONDING AGENTS AND METHODS FOR THEIR USE**

(75) Inventors: **R. Scott Hamilton**, Bear River City, UT (US); **Gary K. Lund**, Ogden, UT (US); **Robert M. Hajik**, Willard, UT (US)

(73) Assignee: **Orbital ATK, Inc.**, Dulles, VA (US)

(\*) Notice: Subject to any disclaimer, the term of this patent is extended or adjusted under 35 U.S.C. 154(b) by 0 days.

(21) Appl. No.: **08/204,044**

(22) Filed: **Dec. 30, 1993**

**Related U.S. Application Data**

(63) Continuation-in-part of application No. 07/945,683, filed on Sep. 16, 1992, now abandoned.

(51) **Int. Cl.**

**C06B 23/00** (2006.01)  
**C06B 29/22** (2006.01)

(52) **U.S. Cl.**

CPC ..... **C06B 23/00** (2013.01); **C06B 29/22** (2013.01)

(58) **Field of Classification Search**

CPC ..... C06B 23/00; C06B 29/22  
USPC ..... 149/19.1, 19.9, 19.4, 19.92  
See application file for complete search history.

(56) **References Cited**

**U.S. PATENT DOCUMENTS**

|             |         |                |                  |
|-------------|---------|----------------|------------------|
| 2,300,998 A | 11/1942 | White et al.   | ..... 260/566    |
| 3,489,565 A | 1/1970  | Kohn           | ..... 96/66      |
| 3,790,416 A | 2/1974  | Dehm           | ..... 149/19     |
| 3,827,780 A | 8/1974  | Labes          | ..... 350/160 LC |
| 3,891,709 A | 6/1975  | Higuchi et al. | ..... 260/584 B  |
| 4,000,023 A | 12/1976 | Oberth et al.  | ..... 149/19.4   |
| 4,016,113 A | 4/1977  | Preston et al. | ..... 260/2.5 AM |
| 4,019,933 A | 4/1977  | Cuksee et al.  | ..... 149/19.4   |
| 4,151,317 A | 4/1979  | Burba et al.   | ..... 427/388 D  |
| 4,226,792 A | 10/1980 | Tajima         | ..... 260/435 A  |

|             |         |                 |                |
|-------------|---------|-----------------|----------------|
| 4,391,660 A | 7/1983  | Corley et al.   | ..... 149/19.9 |
| 4,402,699 A | 9/1983  | Rose et al.     | ..... 8/412    |
| 4,410,376 A | 10/1983 | Bruenner et al. | ..... 149/19.4 |
| 4,491,538 A | 1/1985  | McCoy           | ..... 252/541  |
| 4,493,741 A | 1/1985  | Ducote et al.   | ..... 149/19.4 |
| 4,531,989 A | 7/1985  | Ducote et al.   | ..... 149/19.2 |
| 4,745,135 A | 5/1988  | Thomas et al.   | ..... 521/114  |
| 4,789,691 A | 12/1988 | Matzke et al.   | ..... 521/159  |
| 4,799,980 A | 1/1989  | Reed, Jr.       | ..... 149/19.4 |
| 4,857,071 A | 8/1989  | Anderson        | ..... 8/414    |
| 4,909,954 A | 3/1990  | Palazzotto      | ..... 558/422  |
| 4,915,755 A | 4/1990  | Kim             | ..... 149/19.4 |
| 4,944,815 A | 7/1990  | Consaga         | ..... 149/19.9 |
| 4,971,640 A | 11/1990 | Chi             | ..... 149/19.9 |

**OTHER PUBLICATIONS**

Nakamura et al., "An Infrared Study of the C=N Stretching Frequency in N-Benzylideneaniline Derivatives", *Chem. Pharm Bull.*, vol. 15, No. 5, pp. 585-592, 1967.

Reeves et al., "The Protonation of Benzylideneaniline and it's p- and p-Dimethylamino Derivatives", *Communication No. 2317* from the Kodak Research Laboratories, Rochester, N.Y., vol. 85, pp. 724-729, Mar. 20, 1963.

Ducote, "Amine Salts as AP Bonding Agents", U.S. Army Missile Command Restone Arsenal, Alabama.

*Primary Examiner* — Liam J Heincer

(74) *Attorney, Agent, or Firm* — TraskBritt

(57) **ABSTRACT**

Bonding agents for use in formulating solid propellants are described. The bonding agents have a Schiff base, or Schiff base and hydroxyl or amine functionality. These materials are synthesized by reacting a primary amine with an aldehyde to form a Schiff base. By definition, a Schiff base comprises the reaction product of a primary amine and an aldehyde. In one embodiment of the invention, such a product is produced by the reaction of a polyoxyalkyleneamine (JEFFAMINE®) with p-nitrobenzaldehyde and glycidol. The result is a poly-ether having both hydroxyl and Schiff base functionality. The bonding agents provide superior performance, while avoiding problems, such as ammonia production during processing, encountered when using existing bonding agents. Propellants formulated using these bonding agents have mechanical properties within acceptable ranges.

**27 Claims, 2 Drawing Sheets**



FIG. 1



FIG. 2

## SOLID PROPELLANT BONDING AGENTS AND METHODS FOR THEIR USE

### RELATED APPLICATION

This application is a continuation-in-part of U.S. patent application Ser. No. 07/945,683, filed Sep. 16, 1992 now abandoned and entitled "Solid Propellant Bonding Agents and Methods For Their Use," which application is incorporated herein by this reference.

### BACKGROUND

#### 1. The Field of the Invention

The present invention relates to polyether compounds usable as solid propellant bonding agents and having imine, or imine and hydroxyl functionality. More particularly, the present invention relates to the use of such organic compounds as bonding agents in the preparation of solid propellants.

#### 2. Technical Background

Solid propellants are used extensively in the aerospace industry. Solid propellants have become the preferred method of powering most missiles and rockets for military, commercial, and space applications. Solid rocket motor propellants have become widely accepted because of the fact that they are relatively simple to manufacture and use, and they have excellent performance characteristics. Furthermore, solid propellant rocket motors are generally substantially more simple and reliable than liquid fuel rocket motors. For all of these reasons, it is found that solid rocket propellants are very reliable and economical.

Typical solid rocket motor propellants are formulated using an oxidizing agent, a fuel, and a binder. At times, the binder and the fuel may be the same. In addition to the basic components, it is conventional to add various bonding agents, plasticizers, curing agents, cure catalysts, and other similar materials which aid in the processing and curing of the propellant. A significant body of technology has developed related solely to the processing and curing of solid propellants.

Many types of propellants used in the industry incorporate ammonium perchlorate (AP) as the oxidizer. The ammonium perchlorate is generally incorporated into the propellant in particulate form. In order to hold the propellant in a coherent form, the components of the propellant are bound together by binder, such as, but not limited to, a hydroxy-terminated polybutadiene (HTPB) binder. Such binders are widely used and commercially available. It has been found that such propellant compositions provide ease of manufacture, relative ease of handling, good performance characteristics, and are at the same time economical and reliable. As a result, this type of propellant has become a standard in the industry.

Propellants are generally required to meet various mechanical and chemical performance criteria in order to be considered acceptable for routine use. For example, it is important that the propellant have desired mechanical characteristics which allow it to be used in a corresponding rocket or missile. It is important, for example, that the propellant elastically deform during use in order to avoid cracking within the propellant grain.

If the propellant cracks, burning within the crack may be experienced during operation of the rocket or missile. Such burning in a confined area may result in an increased surface area of burning propellant or increased burn rate at a particular location. This increase in the burn rate and surface area can directly result in failure of the rocket motor due to over pressurization or burn through of the casing.

Accordingly, propellants are typically subjected to standardized stress and strain tests. The typical configuration of

the propellant sample tested is often referred to as a JANNAF Class C specimen. The shape and size of such specimens are standard in the industry. Such specimens are typically placed in an INSTRON® testing apparatus and then pulled until the specimen fails. Data is recorded during such tests and objective measures of stress and strain performance are provided.

In order to make certain that propellant formulations meet the applicable specifications, it is often necessary to employ a bonding agent within the propellant composition. Bonding agents are used in order to help incorporate solid particles into the polymeric binder system. Use of a bonding agent typically improves the stress and strain characteristics of the propellant.

A number of bonding agents are known and conventional. One such bonding agent is Tepanol (tetraethylenepentamine acrylonitrile glycidol adduct). Tepanol has been found to be useful as a bonding agent, and improves the processing characteristics of the propellant formulation. Tepanol is believed to become chemically linked to the polymeric propellant binder. Tepanol also electrostatically coordinates with the remaining ammonium perchlorate after forming a Tepanol perchlorate salt from an acid/base reaction with ammonium perchlorate. Thus Tepanol aids in binding the ammonium perchlorate particles within the propellant matrix. Tepanol is also inexpensive and readily available.

Tepanol, however, also causes difficulty in the formulation of propellant. Tepanol is relatively basic, and in the presence of ammonium perchlorate produces a significant amount of ammonia. This makes it necessary to conduct propellant mixing steps under vacuum, and to mix for long periods of time in order to substantially remove the produced ammonia. These characteristics of Tepanol result in significant disadvantages, such as long mix time, high labor costs, ammonium perchlorate attrition, and may shorten the service life of the propellant.

An alternative bonding agent is known commercially as HX-752 and is available from 3M. HX-752 is an aziridine having the following general chemical structure:



HX-752 is believed to be incorporated into the propellant matrix by ring opening polymerization. HX-752 avoids the production of large amounts of ammonia which plague processes using Tepanol. As a result, some advantages are derived from the use of HX-752.

Even in view of the foregoing, HX-752 is far from ideal as a bonding agent. One significant problem is that of economics. HX-752 presently costs from four to five times as much as Tepanol. Also, the propellant produced when using this material has a relatively high viscosity, which inhibits processing. It is also believed that HX-752 may be a carcinogen. Thus, it can be seen that the cost and chemical characteristics of HX-752 make it a less than ideal bonding agent.

In summary, conventional bonding agents have significant drawbacks. Tepanol is problematic because of its tendency to produce large quantities of ammonia during propellant mixing and the other limitations mentioned above. Alternative

materials, such as HX-752, also present problems including cost and the processing characteristics of the propellant.

Accordingly, it would be an advancement in that art to provide bonding agents which overcame some of the significant limitations encountered using conventional bonding agents. It would be an advancement in the art to provide bonding agents which did not produce significant quantities of ammonia during propellant formulation. It would also be an advancement in the art to provide acceptable alternative bonding agents which were relatively inexpensive. It would also be an advancement in the art to provide such bonding agents which also resulted in propellants having acceptable stress and strain characteristics.

Such compositions and methods are disclosed and claimed herein.

#### BRIEF SUMMARY

The present invention relates to bonding agents which include a Schiff base or a combination of Schiff base and hydroxyl or amine functionality. The compounds of the present invention are found to function well as bonding agents in the formation of solid propellant compositions. The Schiff base, or combination of Schiff base with hydroxyl and/or amine functionality in a single organic molecule, provides the compounds with the ability to serve as effective bonding agents, while avoiding some of the significant problems encountered with conventional materials.

Schiff bases comprise a subgroup of imines. An imine is generally defined as the reaction product of an amine or ammonia and an aldehyde or ketone. This reaction results in a molecule with at least one  $C=N$  group. In that context, it has been discovered that unsubstituted imines formed from ammonia are generally unstable and polymerize on standing. Conversely, if a primary amine is used instead of ammonia, a more stable reaction product is formed. This product is defined as a Schiff base. Therefore, a Schiff base is an imine (having at least one  $C=N$  group) formed by the reaction of a primary amine with an aldehyde or ketone, and preferably in which at least one of the functional residues is aromatic.

It is generally found that aromatic aldehydes or arylamines result in the most stable imines. Other aldehydes or ketones may also be used, and Schiff bases formed from such aldehydes or ketones are to be considered to fall within the scope of the present invention.

The compounds of the present invention have the following general structure:



In the general structure,  $R_1$ ,  $R_2$ ,  $R_3$ , and  $R_4$  may be the same or different and are selected from the group consisting of hydrogen or aliphatic linear or branched alkyls having from 1 to 20 carbon atoms, and more preferably 1 to 10 carbon atoms. At least one of  $R_1$ ,  $R_2$ ,  $R_3$ , and  $R_4$  contains an ether linkage between aliphatic residues. At least one of  $R_1$ ,  $R_2$ ,  $R_3$ , and  $R_4$  contains a Schiff base. In addition, at least one of  $R_1$ ,  $R_2$ ,  $R_3$ , and  $R_4$  may contain a hydroxyl group or an amine.  $W$ ,  $X$ ,  $Y$ , and  $Z$  are selected from the group consisting of free hydroxyl ( $—OH$ ), aromatic imine (Schiff base), hydrogen, or  $CH_3$ . In certain preferred embodiments of the invention at least one of  $W$ ,  $X$ ,  $Y$ , and  $Z$  is hydroxyl and at least one is Schiff base.

One specific example of a compound falling within the scope of the present invention is:



The primary amine employed in preparing the bonding agent of the present invention may be virtually any amine or  $—OH$  containing amine. The amine may be of substantially any carbon chain length and may be branched or unbranched. Other functional groups may also be included on the primary amine molecule, so long as those groups do not interfere with the necessary reaction. Such groups may include ethers and esters.

In order to provide the desired hydroxyl functionality, the primary amine may also be reacted with an epoxide, acrylonitrile, acrylate, methacrylate, or similar molecule capable of imparting hydroxyl functionality to the end product. One such epoxide which provides good results is glycidol; however, a variety of epoxides are capable of providing the same function.

One compound falling within the scope of the present invention is formed by the reaction of polyoxypropylenetriamine (available from Texaco, Co. under the name JEFFAMINE®), with *p*-nitrobenzaldehyde, and glycidol. The product formed from the reaction contains varying amounts of imine and hydroxyl functionality. The reaction is essentially as follows:





10

A general description of one preferred group of bonding agents within the scope of the present invention would include the following general structure:



Where  $\text{R}_1$ ,  $\text{R}_2$ , and  $\text{R}_3$  may be the same or different and are selected from



The compounds produced in this manner have been found to constitute effective bonding agents in the formulation of propellant compositions, particularly ammonium perchlorate-based propellants. When the compounds of the present invention are used as bonding agents, it is possible to avoid cracking of the propellant and undesired burning. At the same time the propellants are found to have suitable stress and strain characteristics and the propellants do not produce excessive quantities of ammonia during mixing.

The compounds of the present invention are believed to result in polar coordination with ammonium perchlorate within the propellant. The  $\text{N}=\text{C}$  group provides a dipole which is sufficient to result in an association with the ammonium perchlorate. At the same time, the existence of isocyanate reactive functional groups (hydroxyl or amine) provides the mechanism for incorporating the bonding agent within the propellant (polymer) matrix.

Accordingly, typical propellants within the scope of the present invention comprise from about 10% to about 20% hydroxyl-terminated polybutadiene (HTPB) binder, from about 0.1% to about 5.0% of the bonding agents disclosed herein, and from about 50% to about 90% ammonium perchlorate (which may be in multiple particle sizes). All percentages are by weight. Other materials may also be included such as fuels (including aluminum), and curing agents such as isophorone diisocyanate.

The compositions of the present invention are to be contrasted with conventional Schiff base-containing chelating agents. The conventional materials have been used to introduce ballistic modifying metal ions into a propellant matrix. The compositions of the present invention, conversely, are metal-free.

#### BRIEF DESCRIPTION OF THE DRAWINGS

In order that the manner in which the above-recited and other advantages and objects of the invention are obtained, a more particular description of the invention briefly described above will be rendered by reference to the appended drawings. Understanding that these drawings only provide data concerning typical embodiments of the invention and are not therefore to be considered limiting of its scope, the invention will be described and explained with additional specificity and detail through the use of the accompanying drawings in which:

FIG. 1 is a graph which plots stress and strain illustrating baseline data and data from multiple samples.

FIG. 2 is a bar graph which plots ammonia in parts per million for multiple samples.

#### DETAILED DESCRIPTION

The present invention is related to bonding agents which function successfully in the formulation of solid propellants. The organic bonding agents employed include a Schiff base, or a combination of Schiff base and hydroxyl or amine functionality. The compounds are generally synthesized by reacting a primary amine with an aldehyde or ketone to form a Schiff base. The amine may also react with an epoxide, acrylonitrile, acrylate, methacrylate, or other reagent capable of providing hydroxyl functionality.

As discussed above, compositions of the present invention have the following general structure:



In the general structure,  $\text{R}_1$ ,  $\text{R}_2$ ,  $\text{R}_3$ , and  $\text{R}_4$  may be the same or different and are selected from the group consisting of hydroxyl ( $-\text{OH}$ ), aromatic imine (Schiff base), hydrogen, or  $\text{CH}_3$ . In certain preferred embodiments of the invention at least one of  $\text{W}$ ,  $\text{X}$ ,  $\text{Y}$ , and  $\text{Z}$  is hydroxyl and at least one is Schiff base.

One specific example of a compound falling within the scope of the present invention is:



In one preferred embodiment of the present invention, such a compound is made by reacting JEFFAMINE® with p-nitrobenzaldehyde and glycidol. As mentioned above, the use of an aromatic aldehyde or ketone results in a more stable and usable compound. In a typical case, about 1 mole of JEFFAMINE® T-403 (available commercially from Texaco), is combined with up to about 3 moles of p-nitrobenzaldehyde, and up to about 3 moles of glycidol.

The reaction may be run in toluene or any other solvent that will allow the reaction to proceed. A water by-product is produced during the synthesis and water may be removed from the reaction mixture by known techniques. For example, azeotropes or drying agents, such as calcium chloride, have been found to be suitable for water removal.

The reaction product is not necessarily uniform, but this fact does not detract from the usefulness of the product. For example, the reacted mixture may include a small percentage of unreacted JEFFAMINE® molecules along with mono-, di-, and tri-imine (Schiff base) reaction products. In addition, the reacted mixture may include mono-, di-, and tri-dihydroxypropyl products.

The polyether-hydroxy-imine compounds produced provide significant improvement over conventional bonding agents so long as the reaction mixture contains compounds containing Schiff base functionality, or a Schiff base along with amine or hydroxyl groups. For example, it has been found that use of the bonding agent at levels below 1%, and even in the 0.15% range, has provided excellent propellants, even when the solids within the propellant exceed about 87%.

Use of the compounds of the present invention as bonding agents provides propellant having good mechanical characteristics. It is found that such propellants have properties similar to those produced using conventional bonding agents, such as Tepanol and HX-752. FIG. 1 is a plot of stress v. strain measurements obtained using the techniques outlined above, wherein JANNAF Class C specimens are placed in an INSTRON® machine for stress and strain measurements. FIG. 1 shows the performance of a "baseline" propellant which is free of bonding agents. FIG. 1 also provides plots of propellants employing a Tepanol bonding agent, HX-752, and a bonding agent within the scope of the present invention.

FIG. 1 dramatically illustrates the improvement in mechanical characteristics over baseline when a bonding agent is employed. In addition, FIG. 1 shows that the use of the compounds of the present invention as bonding agents provides mechanical properties comparable to those achieved by Tepanol and HX-752. As will be discussed in further detail below, the compounds of the present invention provide the marked improvement in mechanical characteristics, while avoiding problems, such as ammonia production, encountered with the conventional bonding agents.

Conventionally, bonding agents are used to link solid particles to the polymer bonding system of a propellant, thus improving the stress and strain properties of the propellant.

The present invention teaches the attachment of a polar moiety (imine) to the overall organic molecular structure (such as a JEFFAMINE® structure). It is presently believed that the imine then attracts and aligns with the ammonium perchlorate by means of a partial electrostatic interaction. This is accomplished by the nature of the Schiff base, i.e., the C=N group has partial charges ( $\delta^+$ - $\delta^-$ ) which are sufficient to align with the polar ammonium perchlorate molecule. In addition, the conversion of the amine to an imine substantially eliminates the problem of ammonia production in the formulation of propellants.

The compounds of the present invention may also include hydroxyl or amine functionality. These functional groups provide a mechanism for incorporation of the bonding agent and solid ammonium perchlorate within the binder matrix. The hydroxyl functionality reacts with the conventional isocyanate curative used in such propellant formulations. Thus, it is possible to incorporate large quantities of solid into the binder, while still maintaining favorable mechanical properties.

The present invention also relates to the propellants formulated using the bonding agents described above. Importantly, the propellants of the present invention are provided with desirable characteristics because of the nature of the inventive bonding agent.

Typical propellants within the scope of the present invention comprise from about 10% to about 20% binder. The binder will typically be a hydroxy-terminated polybutadiene (HTPB), such as R-45M, manufactured by ATOCHEM. 30 Added to the binder is from about 50% to about 90% oxidizer. The oxidizer generally takes the form of solid particulate ammonium perchlorate having varying particle sizes. Typical particle sizes include 400  $\mu$ , 200  $\mu$ , and 20  $\mu$  particles. It is conventional in propellant formulation to combine ammonium perchlorate particles of multiple sizes. 35

Added to these materials is a bonding agent within the scope of the invention. The bonding agent will in general comprise from about 0.05% to about 5.0% by weight of the propellant formulation. In addition, the propellant will likely 40 include a curing agent, such as isophorone diisocyanate, which crosslinks the HTPB polymer. Other materials may also be added, including additional fuels (such as aluminum), processing aids, and other similar types of additives.

Thus, an effective alternative bonding agent is provided.

45 The bonding agent is economical to produce. It is also convenient to use in that it produces relatively small quantities of ammonia during processing. At that same time, the bonding agent is as effective as known bonding agents in improving the mechanical characteristics of the final propellant formulations.

50

## EXAMPLES

The following examples are given to illustrate various  
55 embodiments which have been made or may be made in  
accordance with the present invention. These examples are  
given by way of example only, and it is to be understood that  
the following examples are not comprehensive or exhaustive  
of the many types of embodiments of the present invention  
60 which can be prepared in accordance with the present invention.

### Example 1

65 A compound within the scope of the present invention was synthesized and characterized. The reagents used were as follows:

| Material            | Grams | Moles/Equiv. |
|---------------------|-------|--------------|
| Jeffamine T-403     | 30.00 | 0.1936 eq.   |
| glycidol            | 4.74  | 0.064 moles  |
| 4-nitrobenzaldehyde | 19.34 | 0.128 moles  |

The synthesis occurred in a 300 ml three-neck round bottom flask equipped with a dean-stark trap, condenser, heating mantle, and thermometer. The synthesis was initiated by placing 30 grams of JEFFAMINE® in the flask along with 4.74 grams of glycidol. The resulting mixture was heated to 30° C., and allowed to exotherm to 45° C. after 1/2 hour. 19.34 grams of 4-nitrobenzaldehyde was added in 200 ml. of toluene. The mixture was heated to reflux for two hours or until 2 ml. of water was recovered from the trap. The reaction product was then recovered and dried with sodium sulfate. The sodium sulfate was filtered off, and the toluene was removed by vacuum.

It was found that the material produced comprised a compound having both hydroxyl and Schiff base functionality. In addition, it was found that the material produced worked well as a propellant bonding agent. A stress vs. strain curve for a propellant using this formulation, and other exemplary propellant formulations, is set forth in FIG. 1.

### Example 2

In this Example, compounds within the scope of the present invention were synthesized using the general procedure set forth in Example 1. The following materials in the following amounts were reacted:

| Material        | Grams | Moles/Equiv. |
|-----------------|-------|--------------|
| Jeffamine T-403 | 33.00 | 0.1937       |
| glycidol        | 4.79  | 0.0646       |
| benzaldehyde    | 13.70 | 0.1291       |

The material produced had the following general structure:



The compound produced resulted in markedly decreased amine content, and a resulting reduction in ammonia produced during processing. Table I contains amine reduction data regarding this exemplary material.

In addition, FIG. 2 provides data regarding the production of ammonia during the formulation of a propellant using these exemplary materials as bonding agents. FIG. 2 illustrates the ammonia produced in parts per million in a one gallon mix. Data is recorded for the first through the fourth addition of ammonium perchlorate. Data is provided for propellants using Tepanol, HX-752, and with the bonding agents described in Examples 1 and 2.

It can be seen from FIG. 2 that each of the propellants using the bonding agents of the present invention produced significantly less ammonia than the propellant using Tepanol. The propellants using these bonding agents experienced ammonia production more comparable to that experienced using the expensive HX-752 bonding agent.

Table II sets forth representative data regarding the processing properties of these compounds. In Table II, end of mix viscosity data is provided, along with ammonia concentration prior to curative addition.

TABLE I

|    | Bonding Agent | Active Amine Equiv. (/100 g) | % Amine Reduction |
|----|---------------|------------------------------|-------------------|
| 20 | Tepanol       | 1.28                         | 0                 |
|    | Example 2     | 0.14                         | 89                |
|    | Example 3     | 0.00                         | 100               |

TABLE II

|    | Bonding Agent | EOM VISC* | EOM VISC** | Amm. Conc. (ppm) |
|----|---------------|-----------|------------|------------------|
| 30 | None          | 12        | —          | —                |
|    | Tepanol       | 7         | 2          | 680              |
|    | HX-752        | 11        | 6          | 200              |
| 35 | Example 1     | 14        | 9          | 110              |
|    | Example 2     | 9         | 9          | 250              |
|    | Example 3     | 7         | 7          | 150              |

\*propellant made in 1-pint mixer

\*\*propellant made in 1-gallon mixer

### Example 3

In this Example, compounds within the scope of the present invention were synthesized using the general procedure set forth in Example 1. The following materials in the following amounts were reacted:

| Material        | Grams | Moles/Equiv. |
|-----------------|-------|--------------|
| Jeffamine T-403 | 30.00 | 0.1937       |
| benzaldehyde    | 20.56 | 0.1937       |

The material produced had the following general structure:



The compound produced resulted in markedly decreased amine content, and a resulting reduction in ammonia produced during processing. Table I contains amine reduction data regarding this exemplary material.

In addition, FIG. 2 provides data regarding the production of ammonia during the formulation of a propellant using these exemplary materials as bonding agents. FIG. 2 illustrates the ammonium produced in parts per million in a one gallon mix. Data is recorded for the first through the fourth addition of ammonium perchlorate. Data is provided for propellants using Tepanol, HX-752, and with the bonding agents described in Examples 1, 2, and 3.

It can be seen from FIG. 2 that each of the propellants using the bonding agents of the present invention produced significantly less ammonia than the propellant using Tepanol. The propellants using these bonding agents experienced ammonia production more comparable to that experienced using the expensive HX-752 bonding agent.

Table II sets forth representative data regarding the processing properties of these compounds. In Table II end of mix viscosity data is provided, along with ammonia concentration prior to curative addition.

Thus, it can be seen that the processing characteristics of the propellants falling within the scope of the present invention are excellent when compared with conventional bonding agents.

#### Example 4

In this Example, a propellant was formulated using a bonding agent within the scope of the present invention. The following materials were used in the following weight percentages:

| Material                                | Weight Percentage |
|-----------------------------------------|-------------------|
| R-45M<br>(HTPB mfg. by ATOCHEM          | 12.09             |
| Bonding Agent<br>(from Example 1 above) | 0.15              |
| Aluminum                                | 18.00             |
| Ammonium Perchlorate (200 $\mu$ )       | 48.30             |
| Ammonium Perchlorate (20 $\mu$ )        | 20.70             |
| Isophorone diisocyanate                 | 0.76              |

The propellant was formulated by conventional techniques. It was observed that the propellant had stress and strain measurements well within the acceptable range. Furthermore, only relatively small amounts of ammonia were released during processing.

As mentioned above, FIG. 2 provides data regarding the production of ammonia during the formulation of the propellants using these exemplary materials as bonding agents. Data is provided for propellants using Tepanol, HX-752, and with the bonding agents described in Examples 1, 2, and 3.

It can be seen from FIG. 2 that each of the propellants using the bonding agents of the present invention produced significantly less ammonia than the propellant using Tepanol. The propellants using these bonding agents experienced ammonia production more comparable to that experienced using the expensive HX-752 bonding agent.

Thus, it can be seen that the processing characteristics of the propellants falling within the scope of the present invention are excellent when compared with conventional bonding agents.

Accordingly, it can be seen that the compounds formulated in the manner described in this example provide excellent bonding agents having both Schiff base and hydroxyl functionality. The bonding agents provide good mechanical properties in a conventional propellant, while producing only small quantities of ammonia during processing.

#### Summary

In summary, the present invention provides new methods of providing bonding agents for the formulation of solid propellants. The bonding agents used overcome some of the significant limitations encountered using conventional bonding agents. The bonding agents do not produce significant quantities of ammonia during propellant formulation. The bonding agents are also relatively inexpensive. The bonding agents are believed to provide both electrostatic coordination with ammonium perchlorate, and a degree of polymerization within the propellant matrix in order to bind particles while providing a processable material.

The data presented also clearly illustrates that when the bonding agents are used in a propellant, the propellants have good stress and strain characteristics. Thus, the propellants meet the objective mechanical criteria for use in actual practice.

The invention may be embodied in other specific forms without departing from its spirit or essential characteristics. The described embodiments are to be considered in all respects only as illustrative and not restrictive. The scope of the invention is, therefore, indicated by the appended claims rather than by the foregoing description. All changes that come within the meaning and range of equivalency of the claims are to be embraced within their scope.

What is claimed and desired to be secured by United States Letters Patent is:

1. A method of formulating a solid propellant comprising combining an oxidizing agent, a binder and a bonding agent, the bonding agent comprising an organic molecule having the structure:



## 13

wherein R<sub>1</sub>, R<sub>2</sub>, R<sub>3</sub>, and R<sub>4</sub> are the same or different and are selected from the group consisting of hydrogen and aliphatic linear or branched alkyls having from 1 to 20 carbon atoms, wherein at least one of R<sub>1</sub>, R<sub>2</sub>, R<sub>3</sub>, and R<sub>4</sub> contains an ether linkage between aliphatic residues, wherein at least one of R<sub>1</sub>, R<sub>2</sub>, R<sub>3</sub>, and R<sub>4</sub> contains a Schiff base (C=N), and wherein W, X, Y, and Z are selected from the group consisting of free hydroxyl (—OH), aromatic imine (Schiff base), H, and CH<sub>3</sub>.

2. A method of formulating a solid propellant as defined in claim 1 wherein at least one of R<sub>1</sub>, R<sub>2</sub>, R<sub>3</sub>, and R<sub>4</sub> contains a hydroxyl group and an amine.

3. A method of formulating a solid propellant as defined in claim 1 wherein at least one of W, X, Y, or Z is hydroxyl.

4. A method of formulating a solid propellant as defined in claim 1 wherein at least one of W, X, Y, or Z is a Schiff base.

5. A method of formulating a solid propellant as defined in claim 1 further comprising a fuel.

6. A method of formulating a solid propellant as defined in claim 5 wherein the fuel comprises aluminum.

7. A method for formulating a solid propellant as defined in claim 1 wherein the binder is a hydroxyl-terminated polybutadiene binder.

8. A method for formulating a solid propellant as defined in claim 1 wherein the bonding agent has the following structure:



wherein R<sub>1</sub>, R<sub>2</sub>, and R<sub>3</sub> may be the same or different and are selected from the group consisting of



9. A method for formulating a solid propellant as defined in claim 1 wherein the bonding agent has the following structure:



10. A method for formulating a solid propellant as defined in claim 1 wherein the binder comprises from about 10% to about 20% by weight of the propellant formulation.

11. A method for formulating a solid propellant as defined in claim 1 wherein the bonding agent comprises from about 0.05% to about 5.0% by weight of the propellant.

## 14

12. A method for formulating a solid propellant as defined in claim 1 wherein the oxidizing agent comprises ammonium perchlorate.

13. A method for formulating a solid propellant as defined in claim 12 wherein ammonium perchlorate comprises from about 50% to about 90% by weight of the propellant.

14. A solid propellant comprising an oxidizing agent, a fuel and a bonding agent, the bonding agent comprising an organic compound having the following structure:



wherein R<sub>1</sub>, R<sub>2</sub>, R<sub>3</sub>, and R<sub>4</sub> are the same or different and are selected from the group consisting of hydrogen and aliphatic linear or branched alkyls having from 1 to 20 carbon atoms, wherein at least one of R<sub>1</sub>, R<sub>2</sub>, R<sub>3</sub>, and R<sub>4</sub> contains an ether linkage between aliphatic residues, wherein at least one of R<sub>1</sub>, R<sub>2</sub>, R<sub>3</sub>, and R<sub>4</sub> contains a Schiff base (C=N), and wherein W, X, Y, and Z are selected from the group consisting of free hydroxyl (—OH), aromatic imine (Schiff base), H, and CH<sub>3</sub>.

15. A solid propellant as defined in claim 14 wherein at least one of R<sub>1</sub>, R<sub>2</sub>, R<sub>3</sub>, and R<sub>4</sub> contains a hydroxyl group and an amine.

16. A solid propellant as defined in claim 14 wherein at least one of W, X, Y, or Z is hydroxyl.

17. A solid propellant as defined in claim 14 wherein at least one of W, X, Y, or Z is a Schiff base.

18. A solid propellant as defined in claim 14 further comprising a fuel.

19. A solid propellant as defined in claim 17 wherein the fuel comprises aluminum.

20. A solid propellant as defined in claim 14 wherein the binder is a hydroxyl-terminated polybutadiene binder.

21. A solid propellant as defined in claim 14 wherein the bonding agent has the following structure:



wherein R<sub>1</sub>, R<sub>2</sub>, and R<sub>3</sub> may be the same or different and are selected from the group consisting of



22. A solid propellant as defined in claim 14 wherein the binder comprises from about 10% to about 20% by weight of the propellant formulation.

23. A solid propellant as defined in claim 14 wherein the bonding agent comprises from about 0.05% to about 5.0% of the propellant.

**15**

**24.** A solid propellant as defined in claim **14** wherein the oxidizing agent comprises ammonium perchlorate.

**25.** A solid propellant as defined in claim **24** wherein ammonium perchlorate comprises from about 50% to about 90% by weight of the propellant. 5

**26.** A solid propellant as defined in claim **23** wherein the bonding agent has the structure:



**27.** A propellant comprising from about 10% to about 20% binder, from about 50% to about 90% oxidizer, and from about 0.01% to about 5.0% bonding agent, wherein the bonding agent comprises an organic molecule having the following structure: 20

**16**

wherein R<sub>1</sub>, R<sub>2</sub>, R<sub>3</sub>, and R<sub>4</sub> are the same or different and are selected from the group consisting of hydrogen and aliphatic linear or branched alkyls having from 1 to 20 carbon atoms, wherein at least one of R<sub>1</sub>, R<sub>2</sub>, R<sub>3</sub>, and R<sub>4</sub> contains an ether linkage between aliphatic residues and at least one of R<sub>1</sub>, R<sub>2</sub>, R<sub>3</sub>, and R<sub>4</sub> contains a hydroxyl group, wherein at least one of R<sub>1</sub>, R<sub>2</sub>, R<sub>3</sub>, and R<sub>4</sub> contains a Schiff base (C=N), and wherein W, X, Y, and Z are selected from the group consisting of free hydroxyl (—OH), aromatic imine (Schiff base), H, and CH<sub>3</sub>, and wherein at least one of W, X, Y, or Z is hydroxyl and at least one of W, X, Y, or Z is Schiff base.

\* \* \* \* \*